

## UNITED STATES PATENT OFFICE

2,605,206

## WOOD PRESERVATIVE COMPRISING CHLORINATED PHENOLICS, ANTHRACENIC OILS, AND CREOSOTES

Lucien Rouzet, Paris, France, assignor to Societe des Laboratoires de Recherches pour Applications Industrielles, Paris, France, a corporation of France

No Drawing. Application December 12, 1947, Serial No. 791,458. In France December 30, 1946

5 Claims. (Cl. 167—27)

1

For protecting wood, and especially railway sleepers, pit props, telegraph poles and the like, against weather and attack by moisture, fungus, insects and the like, it has long been customary to impregnate the wood with the so-called creosote oils obtained from the distillation of coal tars obtained from high temperature carbonisation. For the same purpose, it has also already been proposed to use anthracenic oils obtained from the distillation of coal tars (mainly the so-called pressure oils) and also anthracenic cakes or sludges obtained as by-products from such distillation, dissolved, for example, in the oils obtained from the distillation up to 160° C. of the same tars.

I have found, and the present invention is based on the discovery, that certain substances which do not themselves have exceptional fungicidal properties, possess the surprising property of reinforcing the fungicidal properties of numerous antiseptics, and especially those enumerated above, when mixed with these antiseptics in very small proportions of from about 0.2 to 0.5% by weight of the total mixture. Such additives thus enable the same fungicidal effects to be obtained with much smaller quantities of these known impregnating antiseptics.

These substances which augment the power of the known antiseptics, and which are hereinafter designated by the term "booster," are quite numerous but may be defined in general terms as the chloro substitution products of phenols, cresols, naphtols, polyphenols and saturated carbocyclic aliphatic hydrocarbons.

Accordingly, the present invention consists in a wood impregnating preservative comprising a mixture of a known antiseptic and fungicidal product, such as creosote oil or anthracenic oil, with a very small proportion of from about 0.2 to 0.5% by weight of the total mixture of a "booster" substance which reinforces the antiseptic properties of said known product and which consists of a chloro substitution product of a phenol, cresol, naphtol, polyphenol or cyclic hydrocarbon.

Among these various derivatives the following have been found to be particularly effective, namely, parachlorometacresol, trichlorphenol, trichlorcresol, pentachlorphenol, hexachlorcyclohexane, and orthophenylphenol.

These various "boosters" have been proved as effective with compositions such as these used under the name of creosote oils for impregnating railway sleepers, as with anthracenic oils and sludges, and have conferred upon them a greatly

2

increased activity and a greater value in combating the various causes of timber decay.

In accordance with the invention also, the above-mentioned anthracenic oils or dissolved anthracenic sludges or cakes are given improved impregnating properties, and consequently greater efficiency, by mixture with petroleum hydrocarbons, such as kerosene, gas oil or fuel oil, which may be employed in the proportion of about 10 to 60% of the total mixture.

Moreover, an addition of from about 1 to 5% of naphthalene to the mixtures described increases the fixation of the deposit in the ligneous layers. By virtue of its crystallisation in the ligneous cells, the naphthalene contributes to prevent migration of the semi-liquid substances and also absorbs the solids, so that the resistance of a combination to the weather becomes perfect.

For example, highly satisfactory results have 20 been obtained with a solution containing:

10% of anthracenic cakes or sludges obtained from the cooling, filtration or pressure treatment of crude anthracenic oils obtained from 25 the distillation of coal tar,  
3% of naphthalene,  
0.5% of parachlorometacresol,  
36.5% of various diluents or solvents capable of 30 facilitating penetration into the ligneous layers, such as certain petroleum hydrocarbons of the type of fuel oil.

This solution has proved to be as powerful a fungicide and insecticide as the heavy creosote 35 oil of analogous composition commonly used for impregnating railway sleepers.

Very favourable results have also been obtained with mixtures, in various proportions, of a solution such as that specified above and the heavy creosote oil commonly used for impregnation; for example, a mixture of two parts of the solution to one part of creosote oil.

It has also been found that the specified "boosters" exercise a very marked activating 45 influence on other substances than those, i. e., the heavy creosote oils and anthracenic oils or sludges, commonly used for impregnating timber. Thus, certain schist oils derived from the pressure treatment, distillation or carbonisation of bituminous schists, and oils obtained from the distillation of tars derived from the low temperature carbonisation of coal, may be mixed with the specified fungicide "boosters." These mixtures have also proved capable of being added 50 to anthracenic sludges or oils or to creosote oils

obtained from the distillation of coal tars obtained from high temperature carbonisation.

What I claim is:

1. A preservative for impregnating wood which comprises 10% by weight of a coal tar anthracenic cake, 3% by weight of naphthalene, 0.5% by weight of parachlorometacresol, and 86.5% by weight of fuel oil.

2. A preservative for impregnating wood which comprises about 1 part by weight of creosote oil mixed with about 2 parts by weight of a solution comprising an anthracenic coal tar distillation by-product, a chlorinated phenol selected from the group consisting of parachlorometa cresol, trichloro phenol, trichloro cresol, and pentachloro phenol and a petroleum hydrocarbon, which solution contains about 10% by weight of said anthracenic by-product and from 0.2% to 0.5% by weight of said chlorinated phenol.

3. A free-flowing liquid impregnant for preserving wood, which comprises an anthracenic oil, parachlorometaresol and a hydrocarbon solvent, the amount of parachlorometacresol being from about 0.2% to about 0.5% of the total weight of the mixture.

4. A liquid impregnant for preserving wood which comprises at least one member of the group consisting of creosote and anthracenic oils diluted by a hydrocarbon solvent and from about 0.2% to about 0.5% by weight of a member of 30

5. A liquid impregnant for preserving wood which comprises from about 30% to 60% by weight of a petroleum hydrocarbon, from 1% to 5% by weight of naphthalene, from about 0.2% to 0.5% by weight of a chloro-substitution product of a member of the group consisting of parachlorometa cresol, trichloro phenol, trichloro cresol, and pentachloro phenol and the balance selected from the group consisting of creosote and anthracenic oils.

LUCIEN ROUZET.

#### REFERENCES CITED

The following references are of record in the file of this patent:

#### UNITED STATES PATENTS

| Number    | Name     | Date           |
|-----------|----------|----------------|
| 1,162,152 | Flemming | Nov. 30, 1915  |
| 1,469,466 | Vermeire | Oct. 2, 1923   |
| 1,953,413 | Klarmann | Apr. 3, 1934   |
| 2,182,081 | Hatfield | Dec. 5, 1939   |
| 2,296,401 | Perkins  | Sept. 22, 1942 |

#### OTHER REFERENCES

"Bell Laboratories Record," October 1944, volume XXII, number 14, pages 573 to 576.